

April 11, 1961

E. C. GIAIMO, JR  
ELECTROSTATIC PRINTING

2,979,403

Filed Oct. 24, 1958



Fig. 1a.



Fig. 1b.



Fig. 1c.



Fig. 1d.



Fig. 1e.



Fig. 1f.

INVENTOR.  
EDWARD C. GIAIMO, JR.  
BY *J. L. Chittaker*  
ATTORNEY

April 11, 1961

E. C. GIAIMO, JR

2,979,403

ELECTROSTATIC PRINTING

Filed Oct. 24, 1958

2 Sheets-Sheet 2



## 1

2,979,403

## ELECTROSTATIC PRINTING

Edward C. Giaimo, Jr., Princeton, N.J., assignor to Radio Corporation of America, a corporation of Delaware

Filed Oct. 24, 1958, Ser. No. 769,494

7 Claims. (Cl. 96—1)

This invention relates in general to electrostatic printing and in particular to improved methods of and means for the production of reverse electrostatic printing. A reverse print is defined herein as a print having dark areas corresponding to light areas of an original image.

In electrostatic printing it is usual to form a latent electrostatic image by applying an electrostatic charge to the surface of a photosensitive member and selectively dissipating the charge by exposure to a pattern of light and shadow to be recorded. Thus, in one system it is conventional to place a negative polarity electric charge on the surface of a photo-conductor and to form an electrostatic image by exposing the charged surface, optionally through a suitable projection system, to a light image of a document, scene, or other image to be reproduced. The resulting electrostatic image is thereupon developed by dusting it with an electrostatic developer powder which adheres to the charged portions of the surface. In this manner, there is formed a reproduction of the original being photographed or copied.

By the operation just described, it is apparent that there is formed a dust image corresponding to a direct reproduction of the original. Thus, the portions of the original that are white or light in tone are reproduced by the absence of deposited powder, whereas the dark portions of the original are reproduced by a heavy powder deposit. Occasionally, however, it is desired to employ electrostatic printing for the production of reverse or negative images in which the original being produced in itself corresponds to a tone reversal of an original scene or document. For example, if it is desired to make a positive electrostatic print from a conventional photograph negative, it is necessary to reverse the blacks and whites.

According to one present method of electrostatic printing a reverse image is most suitably formed by use of special developer powders. According to this procedure a developer powder consisting of relatively larger carrier particles carrying on their surface fine developer powder particles, is cascaded across the image surface. By proper selection of the surface electrostatic properties of the carrier particles and the developer powder, it is possible to produce a developer which, if desired, may contain positively or negatively charged powder particles. Conventional methods of electrostatic printing produce electrostatic latent images of negative polarity. It is then possible through use of a negatively charged powder in the developer mixture to produce reverse development of the electrostatic latent image. A positively charged developer powder produces a direct image.

A disadvantage of this system of reverse electrostatic printing is that one type of developer powder is required for forming a direct image and a different type of developer powder is required for forming a reverse image. Since the process of electrostatic printing heretofore described lends itself particularly well to rapid and continuous machine printing processes, it would be desirable to find a system wherein a reverse image might be pro-

## 2

vided with minimum additional equipment complexity. Use of a single developer powder for both direct and reverse image production would be highly desirable.

An object of the invention is to provide improved methods of and means for electrostatic printing for producing a reverse visible image from a latent electrostatic charge image.

Another object is to provide improved methods of and means for obtaining a reverse visible image with the same developing powder used for obtaining a direct image from a latent electrostatic charge image.

A further object is to provide an improved method of and means for reversing the charge pattern defining an electrostatic latent image whereby the image may be directly developed to form an electrostatic print corresponding to a photographic reversal of the original exposure.

In general, the objects of the present invention may be accomplished by first forming an electrostatic latent image by usual well known methods and, before applying developer powder, recharging the latent electrostatic image and briefly exposing the surface to a source of uniform illumination. By this means the image configuration is maintained and the charged and uncharged areas are reversed. A reverse visible image is obtained upon developing.

The invention is described in greater detail by reference to the accompanying drawings wherein similar reference characters are applied to similar elements, and in which:

Figures 1a to 1f are partially sectional views of a first apparatus illustrating the steps for carrying out the improved processes of the invention; and,

Figure 2 is a partially sectional view of a second apparatus for carrying out the improved processes of the invention.

Referring to Figures 1a to 1f, in accordance with the invention a suitable photosensitive member 20 including a photoconducting insulating layer or surface 22 is sensitized by charging the surface, or in other words, depositing electrostatic charge on the photoconductive surface. The photosensitive member preferably is placed on a grounded metal backing plate 24 during charging. The photosensitive member may comprise a paper backing 26 coated with zinc oxide in a silicone resin, and is sensitized immediately prior to use by passing across the surface a corona discharge electrode 28 adapted to deposit on the surface negative charge in the order of several hundred volts. The corona discharge member comprises a plurality of three mil corona discharge wires 29, disposed together and spaced about 0.5 inch from each other and from the photoconducting coating 22. The corona discharge wires are connected to a negative voltage source V (not shown). As an example, a negative voltage of 6000 volts produces a corona discharge which will deposit a negative electrostatic charge upon the surface of the photoconducting coating 22. As the photoconducting coating 22 passes beneath the wires 29, a corona discharge issuing therefrom is attracted to the grounded metal backing plate 24 placed behind the paper backing 26 and deposits upon the surface of the coating 22.

The electrostatically-charged or sensitized photoconductive coating 22 is then exposed to an incident electromagnetic radiation image, for example, a light image from a projector 30. The electrostatic charge is lost or reduced in the illuminated areas and retained in the non-illuminated areas to form a latent electrostatic charge image on the surface 22. In prior art operation the photosensitive surface 22 after exposure bears an electrostatic latent image which is passed directly into a development operation. According to the present invention

however, the photosensitive sheet bearing the latent electrostatic image is passed through two additional operations by means of which a reverse visible image is obtained. After the photosensitive member is exposed to the image, it is again sensitized by depositing a second negative electrostatic charge on the surface of the member, as in the previous operation. The photosensitive sheet is then exposed very briefly to a source of uniform illumination, from a light bulb 34 for example.

The result of these operations is an electrostatic latent image containing neutral areas, or areas of substantially low negative charge, corresponding to the areas which had previously been highly charged, and areas of substantially high negative charge corresponding to areas which had previously been discharged. Thus, if a negatively charged photosensitive member has been exposed to a photographic negative, the transparent areas in the photographic negative become highly charged to a negative polarity in the final latent image and the portions of the final latent image corresponding to dark areas in the photographic negative become substantially neutral. This reverse electrostatic latent image is then passed to a development operation in which triboelectrically positive developer powder 36 is applied to the image surface by any of various means and methods such as from a perforated container 38 to produce a visible image 40 corresponding to a reverse electrostatic print. The reverse visible image is now fixed to the photoconductive coating 22 by applying sufficient heat to fuse the powder image to the coating, thereby fixing the developed image 42 thereto. A source of radiant heat may be provided by an electric resistance element 44 connected to a voltage source 46.

Although not intending to be limited thereby, a theory of operation for the described series of operations is proposed. When the surface of the photosensitive layer is initially charged negatively, a corresponding positive charge appears at the interface of the photosensitive layer and the backing material, forming an electric field through the photosensitive layer. The photosensitive layer, which may be zinc oxide in a suitable resin binder, is a non-conductor and acts as a dielectric layer between the charges. On exposure to an image, the resistivity of the dielectric is modulated, becoming more conductive in the illuminated areas than in the non-illuminated areas. This causes the negative surface charges to substantially recombine with the positive charges in the illuminated areas thereby reducing the electrostatic field strength, while a higher electrostatic field is retained in the non-illuminated areas. During the second charging operation a uniform surface charge is again applied to the photosensitive layer. The non-illuminated area then assumes a higher negative charge than the illuminated area due both to the charge remaining after exposure to the image and to the fact that the charge cannot be raised to as high a value in the illuminated areas due to slow recovery of the resistivity of the photosensitive material. The flash of uniform illumination then causes the areas of highest charge those areas which were not illuminated upon exposure to the image to recombine more rapidly than those areas with the lower charge, to form a latent image in which the previously illuminated areas have a higher electrostatic charge than in the non-illuminated areas. On development with triboelectrically positive developer powder a reverse visible image results.

It is also known that in the conventional method of forming a latent electrostatic charge image it is possible to omit the step of first applying an electrostatic charge to the surface of a photoconductive insulating material. A somewhat longer exposure to an image is then required, but this is compensated for by permitting elimination of one of the charging steps. The mechanism of this operation is not completely understood at this time, but is believed to be associated with charge carriers located in discrete states in the forbidden band of a semiconductor.

It has been found that the methods of the present invention may be employed with photoconductors wherein the initial surface charging step is omitted, and reverse visible images may still be obtained.

Figure 2 shows another apparatus utilizing the method of the invention, and comprises a paper backing 26 having a photoconductive coating 22 on one surface thereof passing between and over pulleys 48 and 50. A series of stations for producing reverse visible images by an electrostatic printing process are disposed along the path of the paper and between the pulleys 48 and 50.

At one station the photoconducting coating 22 is provided with a first uniform electrostatic charge on the surface thereof by means of a plurality of corona discharge wires 52 and a metal backing plate 54. The corona charging mechanism is of the same type as heretofore described.

The electrostatically-charged photoconductive coating 22 now passes to a station where it is exposed to an incident electromagnetic radiation image, for example, a light image from a projector 56. The electromagnetic radiation may be derived by any of the methods well known in the photographic art, for example, by projection from a photographic transparency. Upon exposure to the electromagnetic radiation image, the illuminated areas of the photoconducting coating 22 discharge the charge stored on the surface thereof leaving the non-illuminated areas charged. This produces a first latent electrostatic image substantially corresponding to the electromagnetic radiation image.

The photoconducting coating 22 now passes to a station where it receives a second uniform electrostatic charge by means of a corona discharge source, as heretofore described.

The photoconducting coating 22 now passes to a station where it is briefly exposed to a source of uniform illumination from a light source 57 in a shielded enclosure 58, thereby providing a reverse latent electrostatic image. The illumination for this purpose is most conveniently derived from an incandescent lamp, and is chosen to be of the type to which the photoconducting coating 22 is sensitive.

The photoconducting coating 22 now passes to a station where the reverse latent electrostatic image is developed to a visible image according to any of several well known methods. For example, a grounded rotary pole piece 60 of a magnetic structure having spaced parallel inclined elliptical discs 62 along its length faces the photoconductive coating 22 and a fixed magnetic pole piece 64 faces the backing side of the paper opposite the rotary magnetic pole piece 62. A magnetic field is maintained therebetween through an enclosed magnetic field path and across the gap therebetween through which the photoconductive sheet passes. A trough 66 holds a quantity of a developer mix which comprises developer powder particles and magnetic carrier particles in contact with the discs 62. When the discs are rotated in a clockwise position, as viewed in Figure 2, a quantity 68 of developer mix is carried upwardly and swept across the surface of the photoconducting coating 22. Developer powder particles are deposited in selected areas thereby producing a developed powder image 70 on the surface of the photoconducting coating 22 corresponding to the reverse latent electrostatic image.

The photoconductive coating 22 now passes to a station where the developed image is fixed to the coating. For this purpose an electric resistance element 72 is connected to a voltage source V-V (not shown) which radiates heat sufficient to fuse the powder image 70 to the photoconductive coating 22, fixing the developed image 74 thereto. Other methods of fixing such as spraying with an adhesive or solvent vapors and/or pressure may be used.

In the system shown in Figure 2, if the second charging step and the step of briefly exposing the photoconductive surface to a source of uniform illumination are

omitted, as by deenergizing these stations, an electrostatic print corresponding to an original is obtained. By energizing these two stations, a reverse print is obtained.

As discussed heretofore, it is also possible to omit the station in which the first charge is applied to the photoconductive insulating coating 22. When this is done, it is necessary to use a longer image exposure time.

The methods heretofore described may be employed with paper coated with a photoconductive composition of zinc oxide in a silicone resin and also coated with zinc oxide in a silicone resin sensitized with certain dyes such as Rose Bengal or fluorescein. Other sensitizing materials may also be used, but best results have thus far been obtained with Rose Bengal since zinc oxide so sensitized has exhibited the greatest change in resistivity upon application of charge and exposure to light.

One example of a suitable coating composition may be prepared by intimately mixing 100 grams of a French process type white photoconducting zinc oxide with 65 grams of a 60% solution of a silicone resin in xylene (such as G.E. SR-82 marketed by the General Electric Co., Silicone Products Division, Waterford, New York), and 85 grams of toluene. To these materials about .07 gram of Rose Bengal is added. Incorporation of the Rose Bengal presents no processing problems as it is merely added during dispersion of the zinc oxide in the resin solution. Additional data on dye sensitization is described by C. J. Young and H. G. Greig in "Electrofax-Direct Electrophotography Printing on Paper," RCA Review, December 1954, volume 15, No. 4, pages 469 to 484.

The zinc oxides which are suitable are those which are substantially electrically non-conductive in the dark. When exposed to light they should exhibit a surface photoconductivity of a certain level in order to be of practical use for the purposes of this invention. In testing zinc oxides to determine their suitability, it is convenient to express the results of the measurements of the test as surface photoconductivity because substantially all of the light is absorbed in a thin layer at the surface of the zinc oxide. It has been found that the zinc oxide selected should have a surface photoconductivity of at least  $10^{-9}$  ohm<sup>-1</sup>/square/watt/cm.<sup>2</sup> when exposed to radiation having a wavelength of about 3900 Å.

Typical zinc oxides suitable for this purpose include: (1) Florence Green Seal No. 8 marketed by the New Jersey Zinc Company, Palmerton, Pa.; (2) U.S.P. XIV marketed by Mallinckrodt Chemical Works, New York, N.Y.; (3) U.S.P. marketed by Eagle-Picher Sales Company, Philadelphia, Pa.; and (4) Cat. No. Z-53 marketed by Fischer Scientific Company, Division of Eimer and Amend Company, New York 14, N.Y.

After ball-milling to obtain a smooth uniform consistency, the mixture is coated on the surface of a paper web and dried. Any standard coating technique may be used such as flowing, spraying, dipping, spin-coating, or brushing on.

The developer powder particles of the developer mix may be chosen from a large class of materials, for example: zinc, copper, carbon, sulphur, gum copal, gun sandarac, nylon, polystyrene, sealing wax and other natural or synthetic resins or mixtures thereof. The developer powder particles may be coated with a thin layer of a material for the purpose of modifying the physical or electrical properties of the developer powder. It is preferred, however, to use a pigmented thermoplastic synthetic resin.

A preferred developer powder example may be prepared as follows: a mixture comprising 200 grams of 200 mesh Piccolastic resin 4358 (an elastic thermoplastic resin composed of polymers of styrene, substituted styrene and its homologs) marketed by the Pennsylvania Industrial Company, Clairton, Pa., and 12 grams of Carbon Black G marketed by the Eimer and Amend Co., New York, N.Y., are thoroughly mixed in a stainless steel

beaker at about 200° C. The mixing and heating should be done in as short a time as possible. The melt is poured upon a brass tray and allowed to cool and harden. The hardened mix is then broken up and ball-milled for about 20 hours. The powder is screened through a 200 mesh screen and is then ready for use as a developer powder. This powder takes on a positive triboelectric charge when mixed with iron powder.

An effective and practical method for bringing the 10 properly charged developer powder particles to the surface to be developed is called magnetic brush development. The "brush" comprises the developer powder and the iron powder mixed therewith picked up on the end of a magnet. The magnet causes the powder particles 15 to arrange themselves in the well known manner along the lines of force of the magnet to form the fibers of a brush.

The powder mixture is picked up by the magnet and the resultant brush is swept across the negative electrostatic latent image on the surface to be developed. When 20 the brush passes over a charged area and the electrostatic attraction between the charged developer powder particles and the oppositely charged image areas is greater than the attraction between the developer powder and the iron powder, the developer powder is stripped from 25 the brush and adheres quite strongly to the paper, forming the visible image. The iron powder is retained in the brush by magnetic attraction. The developer mix is thus handled and brought into position by magnetic forces, while the visible image builds up under electrostatic forces. The selective effect is very definite.

The magnetic carrier particles of the developer mix 30 may be chosen from a large class of powdered magnetically-attractable materials such as iron, steel, alloys of aluminum, nickel and cobalt and other magnetic materials.

A preferred carrier material for the developer mix of the example consists of "alcoholized iron," that is, iron particles free from grease and other impurities soluble in alcohol. These iron particles are preferably relatively small in size, being in their largest dimension about 0.002 to 0.008 inch. Satisfactory results are also obtained using a carrier consisting of iron particles of a somewhat wider range of sizes up to about 0.001 to 0.020 inch. It is preferred to utilize a permanent bar magnet for providing the magnetic field for maintaining the developer mix in a loose mass as in the magnetic brush. However, other structures may be used, such as electromagnets or other magnetic field producing means.

The exact steps actually employed in making a reverse print on the photoconductive zinc oxide layer sensitized with Rose Bengal are as follows: (1) A paper sheet is sensitized by giving it a blanket negative charge in the dark with a 6 kilovolt corona discharge source; (2) a photographic negative is placed on the sheet and exposed for 2½ seconds to a 100 watt white tungsten lamp located 18 inches from the surface; (3) the photographic negative is removed and another blanket charge applied as in step (1); (4) the sheet now bearing a latent electrostatic image is exposed for about  $\frac{1}{10}$  second with a 100 watt yellow lamp spaced 18 inches from the surface; and (5) a developer powder comprising the Piccolastic resin described above, carrying a positive electrostatic charge, is applied to the surface, thereby forming a reverse visible image. The image is fixed to the photoconductive coating by applying heat thereto, for example, from an infrared lamp or other heat producing means.

What is claimed is:

1. A method of electrostatic printing comprising the steps of applying a first uniform electrostatic charge of one polarity to a surface of a photoconductive insulating layer, projecting a pattern of radiant energy to which said layer is sensitive to provide a second electrostatic image 70 triostatic image, then applying a second uniform electrostatic charge of said one polarity to said surface, briefly flooding said surface with radiant energy to which said

layer is positive to provide a second electrostatic image in reverse configuration with respect to first electrostatic image, and applying an electrostatically charged developer substance to said surface whereby a reverse visible image is produced.

2. A method of electrostatic printing comprising the steps of producing a first uniform electrostatic charge of one polarity upon a surface of a photoconductive material which comprises a photoconductor dispersed in an electrically insulating vehicle, projecting a pattern of radiant energy to which said layer is sensitive upon said surface thereby producing a charge pattern substantially corresponding to said light image, then producing a second uniform electrostatic charge of said one polarity upon the surface of said photoconductive material, briefly flooding said surface with radiant energy to which said layer is sensitive whereby the configuration of the charge pattern of said electrostatic image is reversed, and applying an electrostatically charged developer substance to said surface whereby a reverse visible image is produced.

3. A method of electrostatic printing comprising the steps of passing a first corona discharge of one polarity over a surface of a photoconductive material which comprises a photoconductor dispersed in an electrically insulating vehicle, projecting a pattern of radiant energy to which said photoconductive material is sensitive upon said surface thereby producing a charge pattern substantially corresponding to said pattern of radiant energy, then passing a second corona discharge of said one polarity over the surface of said photoconductive material, briefly flooding said surface with radiant energy to which said photoconductive material is sensitive whereby the configuration of the charge pattern of said electrostatic image is reversed, and applying an electrostatically charged developer substance to said surface whereby a reverse visible image is produced.

4. A method of electrostatic printing comprising the steps of passing a first negative corona discharge over the surface of a photoconductive material which comprises a photoconductor dispersed in an electrically insulating vehicle, projecting a pattern of radiant energy to which said photoconductive material is sensitive upon said surface thereby producing a charge pattern substantially corresponding to said pattern of radiant energy, then passing a second negative corona discharge over the surface of said photoconductive material, uniformly flooding said surface with radiant energy to which said photoconductive material is sensitive whereby the configuration of the charge pattern of said electrostatic image is reversed, and applying an electrostatically charged developer to said surface whereby a reverse visible image is produced.

5. A method of electrostatic printing for obtaining a reverse visible image comprising the steps of uniformly charging the surface of a photoconductive material with a negative corona source, exposing said surface to a pattern of radiant energy to which said photoconductive material is sensitive, then a second uniform charging of said exposed surface with a negative corona source, uni-

formly flooding said photoconductive surface with radiant energy to which said photoconductive material is sensitive, and depositing a finely-divided electrostatically attractive material on said surface whereby a reverse visible image is produced.

6. An improved method of electrostatic printing where-in a reverse visible image is obtained on a surface of a photoconductive insulating material disposed upon a non-conductive backing, which comprises in sequence the steps of a first charging of the surface of said material with a distributed electrostatic charge of one polarity, exposing said surface to a radiant energy to which said photoconductive material is sensitive comprising a pattern of light and shadow to be recorded whereby said charge is reduced in the illuminated areas of said surface leaving an electrostatic charge image thereon, a second charging of the surface of said exposed layer with a distributed electrostatic charge of said one polarity, briefly flooding said layer with uniform illumination to which photoconductive material is sensitive whereby said charge image is reversed in configuration, and applying an electrostatically charged developer to said surface whereby a reversed visible image is produced.

7. A method of electrostatic printing comprising the steps of projecting a light image upon a surface of a photoconducting insulating layer disposed upon a non-conductive backing, said layer comprising a finely-divided photoconductive zinc oxide dispersed in an insulating binder and said light image comprising a pattern of radiant energy to which said photoconductive layer is sensitive then applying a uniform electrostatic charge to said surface, briefly flooding said charged surface with radiant energy to which said photoconducting layer is sensitive, and applying an electrostatically charged developer powder to said surface whereby a reverse visible image is produced.

#### References Cited in the file of this patent

#### UNITED STATES PATENTS

|           |               |                |
|-----------|---------------|----------------|
| 2,690,394 | Carlson       | Sept. 28, 1954 |
| 2,741,959 | Rheinfrank    | Apr. 17, 1956  |
| 2,756,676 | Steinhilper   | July 31, 1956  |
| 2,764,693 | Jacobs et al. | Sept. 25, 1956 |
| 2,808,328 | Jacob         | Oct. 1, 1957   |
| 2,817,765 | Hayford       | Dec. 24, 1957  |
| 2,833,648 | Walkup        | May 6, 1958    |
| 2,845,348 | Kallman       | July 29, 1958  |
| 2,853,383 | Keck          | Sept. 23, 1958 |
| 2,863,767 | Vyverberg     | Dec. 9, 1958   |
| 2,914,403 | Sugarman      | Nov. 24, 1959  |

#### FOREIGN PATENTS

|         |        |               |
|---------|--------|---------------|
| 521,415 | Canada | Jan. 31, 1956 |
|---------|--------|---------------|

#### OTHER REFERENCES

Wainer: Photographic Engineering, vol. 3, No. 1, pp. 12-12 (1952).

Dessauer et al.: Photographic Engineering, vol. 6, No. 4, pp. 252-255.

UNITED STATES PATENT OFFICE  
CERTIFICATE OF CORRECTION

Patent No. 2,979,403

April 11, 1961

Edward C. Giaimo, Jr.

It is hereby certified that error appears in the above numbered patent requiring correction and that the said Letters Patent should read as corrected below.

Column 6, lines 72 and 73, strike out "to provide a second electrostatic image trostatic image" and insert instead -- upon said surface to provide a first electrostatic image ---; column 7, line 1, for "positive" read -- sensitive --.

Signed and sealed this 12th day of September 1961.

(SEAL)

Attest:

ERNEST W. SWIDER

Attesting Officer

DAVID L. LADD  
Commissioner of Patents  
USCOMM-DC